

Patented July 5, 1927.

1,634,792

## UNITED STATES PATENT OFFICE.

MICHAEL G. MINAEFF, OF NEW YORK, N. Y., ASSIGNOR, BY MESNE ASSIGNMENTS, TO THE LARVEX CORPORATION, OF BROOKLYN, NEW YORK, A CORPORATION OF NEW YORK.

### MOTHPROOFING COMPOSITION.

No Drawing.

Application filed June 24, 1924. Serial No. 722,064.

This invention relates to the moth proofing of woolens, more especially after they leave the mill and either before or after they are made into clothing or other articles.

5 In the moth proofing of woolens, it is the aim to impregnate the wool fibers with solutions which will render them immune to the attack of the moth larvae. These solutions generally contain a toxic substance of suitable character, any one of several of which may be employed.

10 Careful study and research have convinced me, however, that although the solution to be used may contain a thoroughly satisfactory toxic substance, it may nevertheless be wholly impractical or inefficient because of the fact that frequently woolens are encountered which repel the moth proofing solution to such extent that proper impregnation of the woolens by such solution does not take place.

15 My observations have convinced me that one of the most important considerations in the moth proofing of woolens is to insure a thorough distribution of the solution throughout the goods under treatment in order that thorough impregnation of such woolens by the moth proofing solution will result.

20 I have experimented with many moth proofing solutions containing compositions which would thoroughly protect woolens against the attack of moth larvae, if it were possible to properly impregnate such woolens with these solutions, but, in many instances, such solutions would not wet the fibers nor impregnate them to the extent necessary to a permanent moth proofing.

25 It is not uncommon to find fibers of woolens covered or coated with different materials such as grease or wax, etc. which interfere with the interaction of the moth proofing solution with such fibers, so necessary to efficient impregnation and durable moth proofing effect. It is therefore essential that aside from the toxic characteristics of the solution such a solution to fulfill practical requirements must have a good wetting power. This wetting power depends upon 30 several considerations. For example, the solution should possess a relatively low surface tension and the interfacial tension between the liquid and the fabrics to be treated should also be relatively low. Furthermore,

the moth proofing solution should have some affinity toward the materials to be treated so that it can attack them, even though slightly, by chemical and physical interaction with the fibers, the coating, or both combined.

35 Aside from these considerations, it should be borne in mind that when treating finished woolens, the moth proofing operation must be carried on in an expeditious manner. In other words, it is important that the moth proofing solution can be applied quickly, as by spraying or sponging, and the goods permitted to immediately dry, in contradistinction to a prolonged treatment such as might be obtained by prolonged immersion. It therefore becomes imperative that the solution be so constituted as to impregnate the fabric immediately upon being deposited thereon, in order to efficiently fulfill commercial requirements.

40 With these considerations in mind, I have concluded that in the compounding of a moth proofing solution, it is of primary importance to insure proper impregnation of the woolens, since unless thorough impregnation is possible proper moth proofing cannot be obtained irrespective as to what toxic substance is used.

45 The object of the present invention therefore is primarily to provide a moth proofing solution which will embody a carrier or vehicle constituted to rapidly impregnate woolens and serving the purpose of conveying or carrying the toxic into intimate physical and chemical cooperation with the woolen fibers in order that effective and durable moth proofing may result.

50 I have found that a very satisfactory carrier or vehicle, well adapted for the wetting of woolens, may be obtained, through employment, as a base, of a solution of an organic colloid or combination of colloids. Such a solution will rapidly impregnate woolens and will carry a moth proofing toxic compounded therewith into intimate physical and chemical interaction with the woolen fibers.

55 In carrying out the invention in practice, it is desirable that the organic colloid solution be stable and any suitable colloid may be employed together with any suitable toxic substance. I have found that organic acids of the fatty acid series and their salts beginning with caprylic acid and upwards,

i. e., those which produce colloidal solutions, are highly satisfactory for employment as carriers of the toxic constituents of the moth proofing solution. Any suitable toxic may be employed in conjunction with any of such acids, but, for the purpose of illustration, it may be noted that a solution of .1% sodium oleate will function very satisfactorily as a vehicle for approximately one 10 percent of sodium fluoride.

Higher concentrations of oleate will produce better carrying effects, but if the concentration is too high the appearance of the treated woolens will be impaired.

I have found it advantageous to use a small percentage of gelatine in admixture with the oleate, in order to impart advantageous stability to the solution, and, in practice, approximately .005% of gelatine 15 will give satisfactory results.

One formula which may be employed, although obviously not the exclusive one embodies: .1% sodium oleate, .005% gelatine; and, 1% sodium fluoride.

I have further found that by adding to this solution a small and definitely determined amount of free organic acid the composition will be improved both from the standpoint of good wetting and also for increasing the permanency of the treatment. For example, the preferred composition, though not the exclusive one, may be as follows: .1% sodium oleate, .005% gelatine, 25 .1% sodium fluoride; and, .001% citric acid.

The strengths or concentration of the above constituents may vary without departing from the invention.

I wish to emphasize that the formulas which have been specifically enumerated are 30 only illustrative and do not define the limits of this invention, which, broadly stated, consists in the employment in a moth proofing composition of an organic colloid solution which serves as a carrier or vehicle to carry

a suitable toxic substance into intimate 45 chemical and physical cooperation with the fabric to be treated. Manifestly, any suitable toxic substance may be employed e. g., any fluoride compound or any arsenic compound or any of the other toxics which will 50 function properly in the protection of the fabric against the ravages of the moth larvæ. For these reasons, it is to be understood that the invention is not restricted to the specific 55 illustrative examples given but that it is as broadly novel as is commensurate with the appended claims.

Having thus fully described the invention, what I claim as new and desire to secure by Letters Patent is:

1. A moth proofing composition containing sodium oleate, gelatine, and a soluble fluoride.

2. A moth proofing composition containing sodium oleate approximately .1%, gelatine approximately .005%, and sodium fluoride approximately 1%.

3. A moth proofing composition containing a soluble organic colloid, a toxic substance, and an organic acid.

4. A moth proofing composition containing a soluble organic colloid, a toxic substance, and an organic acid in a quantity not exceeding .01%.

5. A moth proofing composition containing sodium oleate approximately .1%, gelatine approximately .005%, a soluble fluoride approximately 1%, and citric acid approximately .004%.

6. A moth proofing composition containing sodium oleate approximately .1%, gelatine approximately .005%, sodium fluoride approximately 1%, and citric acid approximately .004%.

In testimony whereof I have signed the foregoing specification.

MICHAEL G. MINAEFF.